

Nov. 27, 1973

J. D. MCKINNEY ET AL  
HYDRODESULFURIZATION PROCESS FOR PRODUCING  
A HEAVY ASPHALTIC FUEL OIL

Filed Dec. 8, 1971

3,775,305

5 Sheets-Sheet 1



—  
EIG  
—

Nov. 27, 1973

J. D. MCKINNEY ET AL  
HYDRODESULFURIZATION PROCESS FOR PRODUCING  
A HEAVY ASPHALTIC FUEL OIL

3,775,305

Filed Dec. 8, 1971

5 Sheets-Sheet 2

FIG. 2



FIG. II



Nov. 27, 1973

J. D. MCKINNEY ET AL  
HYDRODESULFURIZATION PROCESS FOR PRODUCING  
A HEAVY ASPHALTIC FUEL OIL

Filed Dec. 8, 1971

3,775,305

5 Sheets-Sheet 3



FIG. 3



FIG. 4

Nov. 27, 1973

J. D. MCKINNEY ET AL  
HYDRODESULFURIZATION PROCESS FOR PRODUCING  
A HEAVY ASPHALTIC FUEL OIL

3,775,305

Filed Dec. 8, 1971

5 Sheets-Sheet 4

FIG. 5



FIG. 7

Nov. 27, 1973

J. D. MCKINNEY ET AL  
HYDRODESULFURIZATION PROCESS FOR PRODUCING  
A HEAVY ASPHALTIC FUEL OIL

3,775,305

Filed Dec. 3, 1971

5 Sheets-Sheet 5

FIG. 8



FIG. 9



FIG. 10



1

3,775,305

**HYDRODESULFURIZATION PROCESS FOR PRODUCING A HEAVY ASPHALTIC FUEL OIL**  
Joel D. McKinney and John A. Paraskos, Pittsburgh, Pa., assignors to Gulf Research & Development Company, Pittsburgh, Pa.Filed Dec. 8, 1971, Ser. No. 206,083  
Int. Cl. C10g 23/02

U.S. Cl. 208—210

15 Claims

**ABSTRACT OF THE DISCLOSURE**

Asphalt-containing oils are hydrodesulfurized to below a refractory sulfur level without excessively converting the asphalt present by employing a two-stage hydrodesulfurization system with interstage hydrogen sulfide and light oil removal, wherein the average hydrogen partial pressure in each hydrodesulfurization stage is maintained sufficiently high that the average reaction rate constant is improved by a two-stage operation, but sufficiently low so that not less than about 50 percent by weight of the feed is recovered as a product boiling above the I.B.P. of the feed.

This invention relates to a process for the production of crude or residual oils having an especially low sulfur content. More particularly, this invention relates to a hydrodesulfurization process for producing an asphaltic fuel oil having a low sulfur content.

Various processes have been proposed for the desulfurization of petroleum hydrocarbons, and such processes have been highly effective in the removal of sulfur from the relatively lighter distillate fractions that are obtained from the distillation of crude oil. However, crude oil and reduced crude oil fractions contain a heavy, residue fraction boiling above 1040° F. commonly referred to as "asphalt," which renders the oil much more difficult to desulfurize. Asphalt is a generally low-grade material that has been isolated from the crude oil and utilized in road construction. In addition, it has been proposed to treat the asphaltic fraction of crude oil in some manner so as to upgrade this material into a more valuable product such as a fuel oil. However, asphalt, when isolated, is highly viscous and is difficult to process over a catalyst. Moreover, it consists of large molecules of fused, aromatic rings and contains the greatest amount of the total sulfur content of the full range crude on a relative basis. A further problem is that some of the sulfur content of the asphalt is tied up in the interior of the large molecules thereof, rendering the asphalt especially difficult to desulfurize. In addition, asphalt contains metals, principally nickel and vanadium, which readily deposit on desulfurization catalysts tending to deactivate the catalyst. The cumulative effect of such factors is that much more severe conditions in the form of higher temperatures and pressures are required as well as a different type of catalyst in order to remove the sulfur from heavy, asphaltic oils as compared with desulfurization of a distillate oil.

Sulfur is a major contributor to air pollution. Accordingly, certain municipalities, both local and foreign, have placed an upper limit on the sulfur content of fuel oils. In the past, such locales have placed a one percent by weight sulfur limit on heavy fuel oils, but the trend has been to a lower maximum sulfur content, such as 0.5 weight percent. Such limitations have provided a major impediment to the use of heavy asphaltic hydrocarbon oil fractions as fuel oil, since an asphaltic fuel oil having an 0.5 percent sulfur content is not easily obtained from some high sulfur crudes merely by passing the crude oil over a desulfurization catalyst.

2

For reasons previously unappreciated, the sulfur content of a particular asphaltic crude or reduced oil could be reduced to one percent sulfur in a hydrodesulfurization zone, but if the sulfur level was to be reduced below one percent, the desulfurization temperature had to be increased to a point at which excessive hydrocracking to lower boiling materials resulted. Thus, while it had been relatively easy to reduce the sulfur level of such residual oils from 4 to 1 percent by weight of sulfur without incurring excessive cracking of the feed, it is substantially more difficult for a majority of typical feeds to remove more than about 75 percent of the sulfur without excessive hydrocracking. Excessive hydrocracking is undesirable since it unnecessarily consumes hydrogen and produces undesired light products and coke on the desulfurization catalyst. Furthermore, the nature of the resulting product can be altered to the extent that it is not a heavy fuel oil whereas heavy oils generally have a higher heating value than lighter oils.

Alternatives to attempted in-depth desulfurization of such asphaltic fractions have included blending of the asphaltic hydrocarbon oil with essentially sulfur-free middle distillate oils in order to provide a low sulfur-containing fuel oil. Other proposals have involved hydrorefining asphaltic oils, under conditions wherein the asphaltic material is hydrocracked to extinction to produce lower boiling hydrocarbon products.

It would be highly desirable to provide a process for desulfurizing asphalt-containing hydrocarbon oils so as to render them suitable for use as heavy fuel oils without the need for either blending such materials with lighter oils or converting the asphalt content of such oils to lower-boiling products of a completely different nature which would prematurely deactivate the catalyst.

It has now been found that a particular heavy fuel oil containing an asphalt fraction may be produced having a sulfur content below one percent by weight of means of the present invention which comprises a process which involves passing an asphalt-containing or asphaltic, hydrocarbon oil, such as a crude oil or residual oil (a reduced crude) containing more than about one percent sulfur to a first hydrodesulfurization zone under an average hydrogen partial pressure,  $P_{av}^1$ , withdrawing a first effluent from the first hydrodesulfurization zone having a reduced sulfur content relative to the feedstock, said first effluent comprising hydrogen sulfide, a light gas fraction, an oil fraction containing aromatics and saturates, and a higher boiling asphaltic fraction. The oil fraction is referred to as "light oil" to contrast it to the higher boiling asphaltic fraction. The hydrogen sulfide, the light gas fraction, and a low boiling portion of the light oil fraction are separated from the first effluent, and the remaining portion of the first effluent comprising the asphaltic fraction and a higher boiling portion of the oil fraction is passed to a second hydrodesulfurization zone and is desulfurized under an average hydrogen partial pressure,  $P_{av}^2$ . Each hydrodesulfurization zone is provided with a hydrodesulfurization catalyst that is disposed on a non-cracking support. A second effluent is withdrawn from the second hydrodesulfurization zone which provides a heavy, asphaltic fuel oil containing less than one percent by weight sulfur. The average hydrogen partial pressure,  $P_{av}$ , is maintained above the hydrogen partial pressure value at which the reaction rate constant for the first zone would have the same value as the reaction rate constant for the second zone, but sufficiently low that not less than 40 percent by weight of said second effluent boils above the I.B.P. of the feed to said first hydrodesulfurization zone.

$P_{av}$  is defined as follows:

$$P_{av} = \frac{P^1_{av} + P^2_{av}}{2}$$

wherein

$P^1_{av}$  is the average hydrogen partial pressure in the first hydrodesulfurization zone; and

$P^2_{av}$  is the average hydrogen partial pressure in the second hydrodesulfurization zone.

Surprisingly, it has been discovered that by maintaining the average hydrogen partial pressure in each of the hydrodesulfurization zones of a two-stage desulfurization process above a predetermined point, as will be herein-after described, the highly refractory sulfur present in the asphaltic portion of the oil may be effectively removed at a desulfurization reaction rate that is unobtainable when employing a single stage operation.

The removal of a controlled portion of the normally liquid, light oil fraction, which fraction comprises both aromatics and saturates having a boiling point below that of the asphalt fraction contained in the original crude or reduced crude, that is passed along with the asphaltic fraction to the second hydrodesulfurization zone, results in the reduction of the sulfur content of the resulting heavy crude oil more easily and with less catalyst to below one percent, for example, to below 0.5 and 0.3 percent by weight sulfur, than is possible in a single reaction zone. The removal of the light oil fraction inherently removes substantially all the hydrogen sulfide and light hydrocarbons produced in the first stage so that this material does not enter the second stage.

One modification of the present invention involves a process which comprises passing an asphaltic, hydrocarbon feed containing more than about one percent sulfur to a hydrodesulfurization zone in the presence of hydrogen and a light oil fraction comprising aromatics and saturates having a boiling point below the asphaltic portion of the feedstock to said hydrodesulfurization zone, and controlling the amount of said light oil, and thus the amount of aromatics and saturates that are passed to the hydrodesulfurization zone to increase the desulfurization rate and permit the recovery of a heavy, asphaltic hydrocarbon fuel containing less than about one percent sulfur.

Thus, the present invention provides an asphalt-containing heavy fuel oil, which is practically sulfur free, without the need for blending the asphaltic fuel oil with a sulfur-free middle distillate oil in order to obtain an oil having a low sulfur content, although such blending is not precluded in accordance with the present invention.

A still further modification of the present invention relates to a process for controlling the hydrodesulfurization of an asphaltic, heavy oil, which process comprises passing crude oil or residual oil, for example, which oil contains an asphaltic fraction, through a hydrodesulfurization zone in the presence of hydrogen, the oil increasing in aromatic hydrocarbon content as it passes through the hydrodesulfurization zone, controlling the aromatic content of the oil as the oil passes through said hydrodesulfurization zone, and then withdrawing the oil from said hydrodesulfurization zone at substantially the point at which the aromatic content of the oil no longer increases.

The term "asphalt" or "asphaltic" as employed in the present specification is intended to include the resins and asphaltenes present in crude oil. Asphalt can constitute approximately 5 to 30 percent by volume or more of crude oil and has an initial boiling point of about 1040° F. It is obtained in refineries by a propane deasphalting process (solvent extraction), or from the residues obtained from distillation. Asphaltenes are highly aromatic and consist of large molecules of fused aromatic rings and normally contain the greatest sulfur concentration of any constituent of the full range crude. Unlike other crude fractions, asphalt also contains metals, principally nickel and vanadium. Thus, the asphaltenes and resins may be distin-

guished from the remainder of the crude oil, which material comprises "saturates" and "aromatics," by virtue of the solubility of these aromatics and saturates in propane and the insolubility of the asphaltenes and resins in propane.

The propane-soluble "aromatics" include benzenes, naphthalenes, thiophenes, benzothiophene, and dibenzothiophenes as the predominant molecular species, while the "saturates" include the non-aromatic, propane-soluble species, such as the naphthenes, e.g., cyclohexanes, and the paraffins, e.g., dodecane, and sulfur-containing compounds, such as s-butyl mercaptan. Thus, the material commonly referred to as "asphalt" comprises the residue of a propane extraction. On the other hand, resins and asphaltenes are themselves separable by a pentane extraction, by virtue of the fact that asphaltenes are insoluble in pentane, while both resins and oils are soluble in pentane.

It has been proposed to subject crude oil or a reduced crude containing the asphaltene fraction to a hydrodesulfurization reaction in order to reduce the sulfur content of the crude. The crude oil or reduced crude is passed over Group VI and Group VIII metals on a non-cracking support, such as alumina, in the presence of hydrogen and the sulfur level is relatively easily reduced from about 4 to about 1 percent by weight, i.e., a 75 percent sulfur removal. However, after about 75 percent sulfur removal is effected with a particular feed, such as a Kuwait crude for example, the sulfur content of the feed suddenly becomes quite refractory and a great deal of hydrocracking is experienced in order to accomplish additional sulfur removal thereby consuming a great deal of hydrogen and changing the nature of the product. Thus, the point at which the sulfur remaining in the crude oil becomes refractory may vary with the nature of the particular type of crude oil. This point may be easily determined experimentally. As previously mentioned, the asphaltenes consist of large molecules of fused aromatic rings and contain sulfur in the interior of the large molecules, thereby rendering the sulfur extremely difficult to remove. In addition, the asphalt contains all of the metals, such as nickel and vanadium that are present in the crude, and these metals readily deposit on the catalyst tending to deactivate the catalyst and reduce its effectiveness. For these reasons, more severe conditions in the form of higher temperatures and pressures are required to remove more than 75 percent of the sulfur from the asphaltic oil and such severe conditions result in hydrocracking, i.e., a severing of the carbon-carbon bonds of the asphaltene molecule resulting in lower molecular weight materials, rather than desulfurization by splitting carbon-sulfur bonds.

In order to more fully understand the process of the present invention, reference is made to the drawings 55 wherein:

FIG. 1 is a flow diagram illustrating the desulfurization of an asphaltic, reduced crude in two stages;

FIG. 2 graphically illustrates the effect of hydrogen partial pressure in each desulfurization stage upon the desulfurization reaction rate constant;

FIG. 3 illustrates graphically the percent yield of materials boiling above the initial boiling point of the feed to a desulfurization reactor as the average reactor temperature increases;

FIG. 4 graphically illustrates the change in concentration of the aromatic, saturate, asphaltene and resin fractions of an asphalt-containing reduced crude as the degree of desulfurization increases;

FIG. 5 graphically illustrates volume percentages of aromatics and saturates that are removed at various interstage flash points;

FIGS. 6 to 10 are diagrammatic schemes for obtaining a low sulfur, light aromatic-rich fraction from one portion of the feedstock to solubilize and reduce the viscosity

of the solution of asphaltenes and resins present in the residual portion of the feed prior to desulfurization of the asphaltenes and resins.

FIG. 11 graphically illustrates the reaction rate advantage of a two-stage hydrodesulfurization system as contrasted with a single stage operation.

Referring to FIG. 1, a reduced crude such as a 50 percent reduced Kuwait crude which contains the entire asphalt content of the full crude and therefore also contains all of the nickel and vanadium and most refractory sulfur content of the full crude is charged to the process through line 10 and is pumped through line 14, pre-heater 16, line 18, solids filter 20 and line 22 to drum 24. From drum 24 the liquid oil charge is passed through line 26 to feed pump 30.

Liquid from pump 30 is admixed with hydrogen from line 32 and passed through line 34, valve 36, line 38 and furnace 40. Liquid flow valve 36 is disposed in a non-fully preheated liquid hydrocarbon line. Recycled hydrogen along with make-up hydrogen (if desired) are introduced into the liquid charge to the reactor prior to the preheating thereof. Recycled hydrogen is passed through line 42 and valve 44, while makeup hydrogen may be charged through line 46, compressor 48 and valve 50. The recycled hydrogen and any make-up hydrogen are introduced to the relatively cool liquid charge through line 32.

A preheated mixture of liquid charge and hydrogen in line 54 may be passed through a guard reactor (not shown), if desired. An effluent stream from the guard reactor is charged to the main reactor 60 containing catalyst beds 62, 64 and 66. This stream may have a 650° F.+ boiling range, for example.

The hydrodesulfurization catalyst employed in the process of the present invention is conventional and comprises, for example, Group VI and Group VIII metals on a non-cracking support. Thus, the catalyst may comprise nickel-cobalt-molybdenum or cobalt-molybdenum on an alumina support. The alumina may be stabilized with 1 to 5 percent by weight of silica. The preferred catalyst is a nickel-cobalt-molybdenum on alumina containing less than 1 percent silica which catalyst may or may not be sulfided. Magnesia is also a non-cracking support. An especially preferred catalyst comprises a particulate catalyst comprising particles between about  $\frac{3}{20}$  and  $\frac{1}{40}$  inch in diameter, such as described in U.S. Pat. 3,562,800 to Carlson et al., which patent is hereby incorporated by reference. The same or a different hydrodesulfurization catalyst can be employed in each stage.

An essential feature of the present invention is that the catalyst is provided on a non-cracking support, since the process of the present invention is essentially a non-cracking process in that very little material is produced having a boiling point below the initial boiling point of the feed. However, high boiling material in the feed may be cracked to produce lower boiling products still in the boiling range of the feed. Thus, whereas prior processes have employed techniques involving, for example, high silica-containing catalysts, e.g. 10 percent or more silica, to hydrocrack the asphaltenes in the feedstock, the process of the present invention involves mainly the severance of carbon-sulfur bonds of the asphaltenes and resins in order to desulfurize the difficultly desulfurizable asphalt, rather than cracking carbon-carbon bonds, which results in lower molecular weight materials. Of course, sulfur is removed from oils during the present process, but this type of sulfur removal is relatively easy to accomplish. In other words, the cracking of carbon-carbon bonds as in prior processes employing cracking produces a material other than a heavy fuel oil and is outside the scope of the present invention. Thus, a relatively minor amount of material is produced having a boiling point below the initial boiling point of the feed to the hydrodesulfurization unit.

As previously mentioned, hydrogen is introduced along with the feedstock by means of line 32. Conventional reaction conditions in the hydrodesulfurization reactor are employed, for example, a hydrogen partial pressure of 1000 to 5000 pounds per square inch, preferably 1000 to 3000 pounds per square inch, is employed. A hydrogen partial pressure of 1500 to 2500 pounds per square inch is especially preferred. The gas circulation rate may be between about 200 and 20,000 standard cubic feet per barrel, generally, or preferably about 3000 to 10,000 standard cubic feet per barrel of feed, and preferably containing 85 percent or more of hydrogen. The mol ratio of hydrogen to oil may be between about 8:1 and 80:1.

As previously indicated, an essential feature of the present invention is the employment of a predetermined, average hydrogen partial pressure in each of the two hydrodesulfurization zone which will permit the desulfurization of the asphaltic oil of the present invention to the necessary extent without undue conversion of the asphaltenes and resins. It is necessary to employ a sufficiently high hydrogen partial pressure, particularly in the second hydrodesulfurization stage where the removal of the highly refractory, asphaltic sulfur takes place, in order to provide hydrogen to the reactive surface of the asphaltene molecule. It is the chemical activity as expressed in the partial pressure of hydrogen, rather than total reactor pressure, which determines hydrodesulfurization activity.

Referring now to FIG. 2, two curves are shown which relate hydrogen partial pressure to the hydrodesulfurization reaction constant  $k$ , defined as

$$k = \left( \frac{1}{S_p} - \frac{1}{S_f} \right) \text{LHSV}$$

wherein:

$S_p$ =pounds of sulfur per pound of oil in the product;  $S_f$ =pounds of sulfur per pound of oil in the feed; and LHSV=volume of oil per hour per volume of catalyst.

The dashed curve of FIG. 2 illustrates the variation in the desulfurization reaction rate constant of various hydrogen partial pressures for the first hydrodesulfurization stage. As will be hereinafter demonstrated, most of the sulfur removed in the first stage is removed from the non-asphaltic aromatics and saturates, which sulfur is not very refractory. Thus, although the hydrogen partial pressure in the first stage should be above about 1000 to 1400 p.s.i. for the particular feed and catalyst employed, there is little advantage in employing hydrogen partial pressures above 1400 p.s.i.

On the other hand, the solid line curve of FIG. 2 shows the effect of hydrogen partial pressure upon the reaction rate constant in a second stage following a 650° F. flash (corresponding to atmospheric pressure) of hydrogen sulfide, light gases and a light fraction of the aromatics and saturates. At hydrogen partial pressures in the second stage below 1400 p.s.i. (the point where the curves intersect), the reaction rate constant is generally lower in the second stage as compared with the reaction rate constant for the first stage. Moreover, as the hydrogen partial pressure is increased above 1400 p.s.i., the reaction rate constant in the second stage very rapidly outranges the reaction rate constant in the first stage. Accordingly, there is an unexpected advantage of maintaining the average hydrogen partial pressure,

$$P_{av} = \frac{P_1^2 + P_2^2}{2}$$

above the hydrogen partial pressure value at the point of intersection of the two curves, i.e., the point at which the reaction rate constant for the first stage has essentially the same value as the reaction rate constant for the second stage.

While FIG. 2 illustrates the advantage of employing increasing hydrogen partial pressures, a point is reached, in one example, at a hydrogen partial pressure of 2200

p.s.i. where the hydrogen partial pressure becomes significantly high that excessive hydrocracking occurs, since high hydrogen partial pressures induce hydrocracking. Accordingly, the upper hydrogen partial pressure must not exceed 2200 p.s.i. for the system illustrated in FIG. 2. Otherwise, the process becomes a cracking process, rather than a non-cracking process, and with all the attendant disadvantages thereof. Accordingly, the average hydrogen partial pressure of the first and second hydrodesulfurization stages must be sufficiently low that not less than 40 percent by weight of the effluent from the second stage boils above the I.B.P. of the feed to the first hydrodesulfurization stage.

Thus, the process of the present invention provides a yield of not less than 40 or 50 and up to 80 and 90 percent by weight of material having a boiling point greater than the initial boiling point (I.B.P.) of the feed to the first desulfurization reactor. Very little, if any, hydrocracking occurs in accordance with the present invention and the hydrogen consumption will be generally in the range of only 150 to 1500, and preferably in the range of 300 to 1000 standard cubic feet per barrel of feed. The feed to the hydrodesulfurization reactor can have an I.B.P. of not less than 375° F., and will preferably have an I.B.P. of at least 620° or 650° F. Thus, the amount of material obtained from the second hydrodesulfurization stage whose boiling point is lower than 375° F., 620° F., or 650° F. will not exceed 50 or 60 percent by weight, generally or preferably 10 or 20 weight percent. A feed having an I.B.P. greater than 650° F., e.g. vacuum tower bottoms having an I.B.P. in the range of 750 to 900° F. or more, may be employed in the process of the present invention. In that event, the amount of material obtained from the second hydrodesulfurization zone whose boiling point is below 650° F. will not exceed 10 or 20 weight percent.

Likewise, the fuel oil product from each hydrodesulfurization unit has a total asphaltenes plus resins content of at least 10 or 20 and can have 30 or 40 up to 80 percent by weight of that present in the feed to the first hydrodesulfurization unit. The fuel oil product from the second hydrodesulfurization unit has a preferred total content of resins plus asphaltenes of at least 40-50 or 70 up to 90 percent by weight of that present in the feed to second hydrodesulfurization zone. This is a further indication that the resins, and particularly asphaltenes may be desulfurized without their complete destruction as was previously proposed.

The point of intersection of the stage I and stage II curves of FIG. 2 will vary depending upon the catalyst and the feedstock that undergoes hydrodesulfurization. With some catalysts and/or feedstocks, the point of intersection may be as low as 1000 p.s.i., so that effective two-stage operation can occur between 1000 p.s.i. and 2200 p.s.i. Likewise, the point at which excessive hydrocracking occurs may vary both below and above 2200 p.s.i., e.g. 2500, 3000 or 3500 p.s.i.

The data for FIG. 2 was obtained by charging a 4.1 weight percent sulfur-containing Kuwait reduced crude to a first stage to reduce the sulfur content to one percent, and the effluent is flashed at 650° F.+ based on atmospheric pressure. The sulfur content is reduced to 0.5 weight percent in the second stage. The catalyst in each stage is a nickel-cobalt-molybdenum on alumina catalyst.

In certain instances, it is advantageous to employ a higher hydrogen partial pressure in the second stage than that which is employed in the first stage. However, the hydrogen partial pressure in the first stage may be substantially the same as that employed in the second stage, if desired.

Hydrodesulfurization reactor temperatures may range between about 650° and about 900° F., and preferably between about 680° and 800° F.

Referring again to FIG. 1, each succeeding catalyst bed 62, 64 and 66, may have a larger volume than the

bed just prior to it. If desired, there may be 4 to 6 catalyst beds in the reactor and, if desired, each reactor bed may have 25 percent, 50 percent, 100 percent or more catalyst than the bed just prior to it.

As previously mentioned, because there is no guard chamber line 54 will lead directly to the reactor. The effluent in line 54 is joined by a hydrogen stream from line 67, valve 69 line 70 and valve 72 so that a hydrocarbon and hydrogen stream is charged to the top of the reactor through line 74. As previously mentioned, the reactor stream is passed through catalyst bed 62 and due to the exothermic nature of the hydrodesulfurization reaction, it becomes heated in passage therethrough. Temperatures between the various catalyst beds may be controlled by employing a hydrogen quench which may be introduced by means of line 76, valve 78, sparger 80, and line 82, valve 84 and sparger 86. Finally, the reaction mixture passes through catalyst bed 66 and then leaves the reactor with, for example, about a one percent by weight sulfur content.

Referring now to FIG. 3, it is seen that as an asphaltic hydrocarbon crude oil residue containing 4 percent sulfur is passed through a hydrodesulfurization zone, such as reactor 60 in FIG. 1, to produce a 1 percent sulfur-containing 660° F.+ product, well over 80 percent of the product boils at 660° F. or above (the initial boiling point of the feed) as the average reactor temperature is increased to compensate for catalyst aging. However, when the reaction temperature is raised to 800° F., excessive hydrocracking to lower boiling materials results. This causes a drop in the curve as to the materials boiling below the initial boiling point of the feed. At this point excessive hydrocracking occurs in order to produce a 1 percent sulfur-containing 660° F.+ product.

As will be hereinafter demonstrated, the process of the present invention permits the efficient removal of greater than 75 percent sulfur from an asphaltic oil and overcomes the refractory nature of such oils.

Reference is now made, once again to FIG. 1. Next, the effluent in line 88 is passed to a high pressure flash chamber 90 wherein light hydrocarbon gases, hydrogen sulfide, hydrogen and a controlled portion of the relatively highly desulfurized saturates and aromatics are removed by means of line 92. The operation of this intermediate flash chamber 90 constitutes a critical feature of the present invention. By carefully selecting the flash temperature at the process pressure, the proper amount of light oil, which is to be removed from the feedstock to the second hydrodesulfurization feed stream is determined. The reason for the removal of an amount of light oil will be demonstrated by reference to FIG. 4.

Referring now to FIG. 4, the composition of a 650° F.+ hydrocarbon oil containing various proportions of aromatics, saturates, resins and asphaltenes is presented, as the oil is passed through a hydrodesulfurization reactor, such as reactor 60 of FIG. 1. As shown in FIG. 4, the resins and asphaltenes content of the feed steadily decreases with increasing sulfur removal due to the severing of carbon-sulfur bonds thereby breaking off molecular fragments. The accumulation of these molecular fragments is reflected in the build-up of lower molecular saturates and aromatics and particularly aromatics. This increase in aromatics content in the liquid is beneficial because the aromatics constitute a solvent for the highly viscous resins and asphaltenes, whereas the resins and asphaltenes are not solvated by saturates. The desulfurization of each fraction continues until about 75 percent sulfur removal, and at that point the resins and aromatics curves reach a plateau which indicates no further cracking of fragments therefrom. At the same time, the total aromatics and saturates content does not increase further, but an increase in saturates level is accompanied by a decrease in aromatics level. This indicates that at 75 percent sulfur removal the aromatics tend to become saturated, which represents not only a fruitless consump-

tion of hydrogen, but deprives the remaining resins and asphaltenes of aromatic solvent, while merely increasing the amount of saturates, which is a mere dispersent.

At the 75 percent sulfur-removal level, the sulfur becomes refractory to further desulfurization so that further desulfurization is accompanied by a loss in aromatics and a sharp increase in saturates. Both of these factors are detrimental in regard to removing further sulfur and overcoming the refractory nature of the oil at this point, since at the 75 percent sulfur-removal level most of the unremoved sulfur is concentrated in the resins and asphaltenes. Thus, a loss of aromatics deprives the viscous resins and asphaltenes of some solvation, while the formation of saturates imparts an excessive dispersion to the system tending to excessively dilute the remaining sulfur and thereby lower the reaction rate.

Thus, while operating the first hydrodesulfurization reactor, the aromatic content of the oil can be measured as it passes through the reactor, and the oil should be withdrawn from the reactor when the aromatic content of the oil is no longer increased. This was the situation at 75 percent desulfurization in FIG. 3. The aromatic content can increase 25 to 40 percent by weight or more as it passes through the reactor. Even a small increase in aromatics concentration is beneficial, e.g. 2 to 5 or 10 percent by weight. Of course, the aromatics concentration should not increase to such a great extent that it unduly dilutes the sulfur which is to be removed.

Without attempting to limit the present invention to any particular theory or mechanisms, it is believed that up to the 75 percent sulfur removal there is a removal of fringe sulfur from the complex heterocyclic ring structure of the asphaltene molecule accompanied by an in situ production of aromatic hydrocarbons mainly due to a severing of the carbon-sulfur bonds on the fringe aromatic rings. This production of aromatics is important, since asphaltene molecules have a tendency to form colloidal crystallites or aggregates, if the molecules are poorly solubilized. Thus, up to the 75 percent sulfur removal level, there is sufficient in situ production of aromatics to solubilize the asphaltene particle and permit contact of the internal, heterocyclic sulfur with the hydrogen and catalyst necessary to desulfurize the asphaltene. However, at the 75 percent desulfurization level, the ratio of aromatics to saturates is sufficiently small that there is insufficient solvent and too much diluent to effect the removal of the refractory sulfur.

For this reason, it is necessary to control the aromatic content of the asphaltic feed to the second hydrodesulfurization zone. This may be accomplished by flashing or otherwise separating, e.g. by distillation or flashing followed by partial condensation of flashed hydrocarbon and recycle, a controlled portion of the normally liquid effluent oil from the first desulfurization zone to provide the proper aromatics content to the stream.

Thus, it is essential to include sufficient aromatics in the feed to the second desulfurization reactor to solubilize the resins and asphaltenes in the oil and to deagglomerate any asphaltene aggregate which may be formed. At any given flash temperature, the removal of a particular quantity of aromatic hydrocarbons normally removes an even greater quantity of saturated hydrocarbons. With certain crudes the flash may remove more aromatics than saturates, in which case the benefit of the flash will be derived from removal of excess dispersent. A compromise must be reached wherein sufficient aromatics are charged along with the feed to the second hydrodesulfurization stage so that the resins and asphaltenes are adequately solvated in order to permit proper desulfurization of the resins and asphaltenes, without the quantity of aromatics being so high that the total aromatics and saturates fed to the second stage will excessively dilute and disperse the sulfur to be removed and thereby reduce the reaction rate. The volume

of aromatics and saturates, respectively, which may be removed at a given flash point is shown in FIG. 4.

Referring now to the solid lines of FIG. 5, an analysis of the saturate and aromatic content of the first sulfur removal stage effluent is shown for various flash points when measured at atmospheric pressure. Thus, if the interstage flash point is 500° F., all of the aromatics boiling above 500° F. will enter the second stage and will be available for solvating the resins and asphaltenes. However, at 500° F., the stream comprises about 81 percent by volume saturates and about 19 percent by volume aromatics. This amount of aromatics together with the even greater amount of saturates which necessarily accompany it, might excessively dilute the asphaltic compounds and thereby lower the reaction rate. On the other hand, if the interstage flash point is as high as 800° F., the oil fed to the second stage will have a higher ratio of aromatics to saturates which is desirable in order to accomplish high solvation with minimum dilution. However, at the 800° F. flash point, the total amount of aromatics which enter the second stage may not be great enough to dissolve the resins and asphaltenes and to sufficiently lower their viscosity to permit desulfurization. Accordingly, a proper balance of aromatics to saturates must be employed in order to obtain optimum desulfurization. This point may be easily experimentally determined for a particular stream undergoing desulfurization. For example, employing as a feed the residue represented by the overhead designated by the solid lines of FIG. 5, the best results are obtained by flashing at the temperature which gives about a 650° F. separation regardless of the elevated pressure of the flash. This provides not only sufficient total amount of aromatics in the stream, but a ratio of about 72 percent saturates by volume to about 26 percent aromatics in the overhead. As will be hereinafter demonstrated, the employment of an excessive amount of aromatics in the desulfurization reaction can be as detrimental to sulfur removal as employing too little aromatics.

The dashed lines of FIG. 4 designate another possible overhead saturates and aromatics distribution in which aromatics begin to predominate in a 550° F. overhead fraction. However, since a 550° F. flash includes all the lighter material, the total overhead will still predominate in saturates over aromatics.

Referring again to FIG. 1, a predetermined amount of liquid is flashed and removed by means of line 92. Depending upon the nature of the feedstock employed and the conditions utilized in the desulfurization reaction, the flashed material in line 92 may contain, for example, between about 5 and about 60 percent by weight of the liquid effluent from the desulfurization reactor 60, preferably between about 10 and about 35 percent by weight. Suitable flash temperatures include, for example, between about 500° and about 800° F., preferably between about 600° and about 700° F. (These temperatures refer to atmospheric pressure and of course will be different at the process pressure). An especially preferred flash point for the interstage flash is 650° F. The most desirable amount of liquid to be flashed or otherwise separated from the desulfurization effluent stream may be easily determined experimentally. The flashed material in line 92 is passed to a high pressure flash chamber unit 94 wherein hydrogen, hydrogen sulfide and light hydrocarbon gases are separated from a liquid hydrocarbon fraction. The gases are withdrawn by means of line 96 and are subjected to purification and separation, including various scrubbing operations and the like in recycle gas recovery unit 97. Subsequently, all of the hydrogen sulfide that it produced in reactor 60 is removed by means of line 93. Hydrogen now free from hydrogen sulfide and light hydrocarbon gases is recovered from unit 97 and is passed by means of line 99 to recycle gas compressor 101 and recycled for utilization in the process

by means of line 103. The non-flashed liquid fraction is discharged from flash unit 94 by means of line 98.

The bottoms fraction from the flash unit 90 is discharged by means of line 100 and is admixed with make-up hydrogen, which is provided by means of line 102, valve 105 and line 107. In addition, recycle hydrogen may be added to the make-up hydrogen in line 107 from line 103 by means of line 109, valve 115 and line 113. If desired, make-up hydrogen may be passed from line 103 directly to line 108 by appropriate valving (not shown). The combined stream may be charged to a furnace 106 in order to raise the temperature of this stream if desired. However, furnace 106 is optional, as the stream 104 may be already at the desired desulfurization temperature for introduction by means of line 108 to the second hydrodesulfurization reactor 110.

The temperatures and pressures employed in reactor 110 may be the same as those described for the hydrodesulfurization reactor 60. Likewise, the desulfurization catalyst which is employed in reactor 110 may be identical to that described previously for reactor 60. It is noted at this point that the hydrodesulfurization catalyst is even more active for removal of nickel and vanadium than it is for removal of sulfur. Most of these metals will be removed in the first hydrodesulfurization reactor 60. The heaviest laydown of such metals is at the inlet to reactor 60. The second desulfurization reactor 110 will act as a metals clean-up stage, and the catalyst therein will not collect as much metals as does the catalyst in reactor 60. Hence, the first stage catalyst will remove most of the metals and will become deactivated by metals much faster than the second stage catalyst.

The desulfurized effluent from reactor 110 is discharged by means of line 114 and is passed to a flash unit 116 for removal of light gases including hydrogen, hydrogen sulfide and light hydrocarbons. This gaseous stream is sent by means of line 118 to high pressure flash unit 94. Meanwhile, a bottoms fraction including the asphaltic product stream of the present invention is passed by means of line 120 to a distillation column 122. A sulfur containing stream comprising sour gas and sour water is removed from column 122 by means of line 124. This stream is passed to a gas treatment plant (by a means not shown) to recover sulfur therefrom. A naphtha fraction is withdrawn from the column 122 by means of line 132. This naphtha stream may be employed as a wash liquid for the separation of the light hydrocarbons from the hydrogen in line 96 (by a means not shown). A furnace oil or heavier fraction may be withdrawn through line 133 and be employed in a manner hereinafter described to provide additional aromatics to the second stage desulfurization reactor 110. A product stream 134 is discharged from the distillation column 122. This desulfurized oil stream contains asphaltenes and resins, and is especially useful, without further blending, as a fuel oil, particularly since less than one percent by weight sulfur is contained therein. Thus, this heavy, asphaltic fuel oil contains, for example, between about 0.3 and about 0.5 percent by weight sulfur or less, which is well within the requirements of even the strictest ordinances for sulfur content of heavy fuel oils.

A modification of the process shown in FIG. 1 is illustrated in FIG. 6, which is a simplified schematic diagram.

Referring now to FIG. 6, a reduced crude oil is introduced by means of line 220 to an atmospheric distillation unit 222 wherein a light asphalt-free distillate fraction having a 630°-650° F. end point (E.P.) is withdrawn by means of line 224, while a heavy asphalt-containing 630°-650° F. + fraction containing 4 percent sulfur is discharged by means of line 226 from the distillation column 222. The asphalt-containing bottoms fraction 226 is passed to a vacuum distillation unit 228 wherein additional light oil is discharged by means of line 230 and is admixed with the lighter fraction in line 224 and intro-

duced along with hydrogen from line 233 into a hydrodesulfurization zone 232 by means of the line 234. Zone 232 may be operated with a conventional gas oil desulfurization catalyst but at a lower temperature and hydrogen pressure (e.g., below 1000 p.s.i.) than are employed for the desulfurization of an asphaltic oil. The asphalt-free distillate is easily completely desulfurized in the zone 232 and is discharged by means of line 236 and passed to distillation unit 238 from which an overhead fraction containing hydrogen, hydrogen sulfide and light gases is removed by line 240 and processed as previously described to recover hydrogen and light hydrocarbons.

An aromatic-rich, furnace oil and higher fraction is discharged from the distillation unit 238 by means of line 244. Meanwhile, an asphalt-containing oil is withdrawn from the vacuum distillation unit 228 by means of a line 246. This stream may have, for example, an initial boiling point of about 1000° F. and contain about 5.5 percent by weight sulfur. The stream 246 is passed through a blending zone 250 wherein the asphalt-containing stream is admixed with a controlled portion of the aromatic-rich fraction from the line 244 in order to obtain the desired viscosity and solvency for the asphaltenes and resins contained in the stream. Then hydrogen is added through line 248. The heaviest product from distillation unit 242 can be blended with the product 268, if desired.

Next, the asphaltic fraction containing solubilized resins and asphaltenes is passed by means of line 252 to a first hydrodesulfurization zone 254 and subjected to desulfurization under the conditions previously described in regard to the reactor 60 of FIG. 1. The effluent from zone 254 has a reduced sulfur content and is passed by means of line 256 to an interstage flash unit 258 wherein hydrogen, hydrogen sulfide, light hydrocarbon gases, and a controlled portion of aromatics and saturates is discharged by means of line 260. As previously discussed, a flash point is selected so as to optimize the amount of aromatic solvent available for solubilizing the asphaltenes and resins in the feed to the second hydrodesulfurization zone. An effluent stream 262 is discharged from the flash unit 258 and is admixed with hydrogen which is introduced by means of line 264. The combined hydrogen-oil stream is passed to a second hydrodesulfurization unit 266 wherein the sulfur content of the asphaltic oil is reduced to below one percent by weight. The heavy oil product stream is discharged from the second hydrodesulfurization unit 266, which unit is operated in the manner described for unit 110 in FIG. 1, and is withdrawn by means of the line 268 and treated as previously described for separation of hydrogen sulfide, light gases and the like.

Thus, the system of FIG. 6 provides a parallel mode of operation wherein an initially-separated lighter portion of the crude is desulfurized and is utilized to provide the desired viscosity and solvency for desulfurization of the heavy, asphaltic portion of the crude oil.

Another modification of the FIG. 1 process is illustrated in FIG. 7. Referring now to FIG. 7, an asphaltic oil is introduced by means of line 320 to a distillation unit 322 for separation into an aromatic-poor fraction on which is withdrawn from unit 322 by means of line 324 and an aromatic-rich fraction containing 4 percent sulfur. An aromatic-rich asphaltic oil is discharged from unit 322 by means of a line 326. For example, distillation unit 322 may be operated to provide an asphaltic fraction having an initial boiling point of about 650° F.

The asphaltic stream in line 326 is admixed with hydrogen which is introduced by means of line 328 and the combined stream is passed by means of line 330 into a hydrodesulfurization unit 332 which is operated in the manner previously described. The effluent from zone 332 is withdrawn by means of line 334 and is introduced into a high pressure flash unit 336 where, for example, material boiling below 800° F. is discharged by means of line 338. Accordingly, an asphaltic oil having a boiling point

of 800° F. + is discharged from the flash unit 336 by means of the line 340.

Referring momentarily to FIG. 5, it is seen that at an 800° F. flash point there is a relatively high aromatic to saturate ratio. However, the total aromatic content of the oil at this point may be less than desired. Accordingly, a controlled amount of an aromatic-rich fraction is introduced into the stream in line 340 by means of line 342 in order to provide the resins and asphaltenes with a proper degree of solvency. The combined stream is then admixed with hydrogen, which is introduced by means of line 344 and introduced into hydrodesulfurization reactor 346 where the sulfur level of the asphaltic fuel oil is reduced to below one percent by weight.

The effluent from zone 346 is removed by means of line 348 and is introduced into distillation unit 350 where an aromatic-rich fraction is separated and recovered by means of line 352. A controlled portion of the material in stream 352 is recycled by means of line 342 for admixture with the asphaltic stream in line 340 as previously described. The light gases are discharged from distillation unit 350 by means of line 354, while a substantially sulfur-free, asphaltic, heavy fuel oil is recovered from line 356. Substantially all of the asphaltenes and resins fed to distillation unit 350 are recovered in line 356 with the asphaltic fuel oil. The recycle stream 342 is devoid of asphaltenes. The asphaltenes are not recycled to the first hydrodesulfurization zone, since they would deactivate the catalyst prematurely. They are not recycled to the second hydrodesulfurization zone, since they have already been desulfurized, such recycle would serve no useful purpose.

In the foregoing manner depicted in FIG. 7, a light, desulfurized, aromatics-rich solvent for the asphaltic material is obtained from the product stream.

Still another modification of the present invention is shown in FIG. 8, wherein an asphaltic feed stream is introduced by means of a line 420 to a distillation unit 422 to reduce the feed and prepare a hydrodesulfurization feed for passage through line 426. The asphaltic fraction is discharged by means of the line 426 from unit 422 and is admixed with a controlled portion of an aromatic-rich stream which is introduced by means of line 428. The stream in line 428 can be an aromatic-rich fraction boiling within the range of between about 400° and about 1050° F., preferably between about 650° F. and about 900° F. The combined stream is admixed with hydrogen, which is introduced by means of line 430, and a stream having a boiling point of about 650 F. + and containing about 4 percent by weight sulfur is introduced by means of line 432 into hydrodesulfurization zone 434.

This unit may be operated at a temperature of 690°-790° or 800° F. An effluent stream having a sulfur content of about one percent by weight sulfur is introduced by means of line 436 into flash unit 438. A light oil and gas fraction containing substantially all of the hydrogen sulfide produced is flashed from the unit 438 and discharged by means of the line 440, which stream may have, for example, a 650° F. E.P.

An asphaltic stream having a boiling point of, for example, 650° F. + is admixed with hydrogen which is introduced by means of line 442 and introduced by means of line 442 and introduced by means of line 444 into second hydrodesulfurization zone 446, which may be also operated at about 690° to 790° or 800° F. The effluent from the second desulfurization zone 446 has a sulfur content of less than one percent and is passed by means of line 448 to distillation unit 450. An aromatics-rich fraction is withdrawn from unit 450 by means of line 452 and is recycled by means of line 428 for admixture to the asphaltic oil feedstock to the first desulfurization zone 434. Hydrogen sulfide and light gases are withdrawn from the distillation unit 450 by means of line 454, while a low sulfur asphaltic fuel oil is recovered by means of line 456. Excess from stream 452 not recycled can be

blended with product in line 456 to reduce the sulfur content of the product.

Thus, the arrangement of FIG. 8 utilizes a low sulfur aromatic-rich product stream for solubilizing the asphaltenes and resins in a heavy desulfurization feedstock having a relatively high I.B.P.

A modification of the system of FIG. 8 is shown in FIG. 9.

The process of FIG. 8 is similar to FIG. 9, however, as shown in FIG. 9, the effluent from flash unit 438 that is withdrawn by means of line 440 is passed to a flash unit which is provided with cooling coils. Hydrogen sulfide and light gases are removed in this lower temperature flash, which gases are withdrawn by means of line 443. The remaining heavier effluent is withdrawn from the flash unit 441 by means of the line 445 and is passed by means of pump 447 for admixture with stream 444 for introduction into the second stage desulfurization unit 446.

The mode of operation of FIG. 9 permits the employment of a flash temperature for unit 438, which temperature may be the same as that employed in the hydrodesulfurization units 434 and 446. At the same time the lower temperature flash unit 441 which is provided with cooling coils permits the separation of hydrogen sulfide and light gases and the reintroduction of a material having the optimum aromatics content and initial boiling point.

Thus, for example, if it were determined that the optimum interstage flash temperature corresponded to 650° F. at atmospheric pressure and the desulfurization units 434 and 446 are being operated at about 700° F., the flash unit 438 may also be operated at 700° F. However, the lower temperature flash unit 441 is operated at 650° F. and thus permits the return by means of the 650° F. + material by means of line 449.

Thus, the modification of FIG. 9 avoids the need for reducing the temperature of the stream in line 436 and the reheating of stream 444.

Referring now to FIG. 10, an asphaltic, sulfur-containing, hydrocarbon oil is introduced by means of line 520 to distillation unit 522 for separation of the feed into light gases, which are withdrawn by means of line 524, and an aromatic-rich fraction, which is discharged by line 526, which is to be employed in a manner herein-after described. This aromatic-rich fraction may have a 650° F. E.P.

An asphaltic bottoms fraction having an initial boiling point of, for example, about 650° F. is discharged by means of line 528 and is admixed with hydrogen from line 530 prior to introduction into first desulfurization zone 532. The desulfurized effluent from zone 538 is introduced by means of line 534 into flash unit 536. As before, the optimum flash point has been previously determined and a light oil fraction containing saturates and aromatics is flashed off along with light gases and hydrogen sulfide by means of line 538.

The asphaltic oil is passed from the flash unit 536 and mixed with hydrogen from line 540 and introduced by means of line 542 to the second stage desulfurization zone 546. In addition, the asphaltic feed to the zone 546 is admixed with the aromatic-rich stream 526. Thus, the distillation operation unit 522 is conducted under conditions so that the stream 526 has a selected boiling range and aromatics content which provides maximum solvation for the asphaltenes present in the feed to the second desulfurization zone 546. The effluent from zone 546 is discharged by means of the line 548 and is passed to distillation unit 550 for separation of the asphaltic fuel produced therefrom by means of line 552. Light gas stream 554 and naphtha stream 556 are recovered and treated as usual.

Referring now to FIG. 11, the desulfurization reaction rate constant in the first and second hydrodesulfurization stages is compared with the desulfurization reaction rate constant for a single stage hydrodesulfurization opera-

tion for the same total degree of desulfurization as a function of time. As illustrated in FIG. 11, the relative inefficiency of operating a single stage hydrodesulfurization unit down to 0.5 percent sulfur is demonstrated. On the other hand, when the first stage is operated down to a 1 percent sulfur and the second stage is operated from a 1 percent level down to 0.5 percent sulfur, the desulfurization constant is maintained above that of the single stage process for each stage of the two-stage process.

In addition, it has been found that the average two-stage catalyst aging rate is about two units per day as compared with a single stage aging rate of about 3.5 units per day. Catalyst aging is evidenced by the amount of temperature increase required to produce a constant desulfurization, as metals and coke increasingly coat the catalyst surface with time.

The following examples are presented to further illustrate the invention.

#### EXAMPLE 1

An asphalt-containing, reduced crude oil containing about 4.09 weight percent sulfur and hydrogen are introduced into a hydrodesulfurization zone containing a nickel-cobalt-molybdenum catalyst disposed on a non-cracking, alumina support. The hydrodesulfurization operation is conducted at temperatures of about 650-820° F. and a hydrogen partial pressure of 2000 p.s.i.g., and the resulting asphaltic material is flashed at a temperature corresponding to 650° F. at one atmosphere so as to optimize the amount of aromatics and saturates present in the effluent. The 650° F.+ asphaltic fraction that is withdrawn from the flashing unit has a sulfur content of about 1.09 weight percent sulfur and is introduced into a second hydrodesulfurization zone where the desulfurization is also conducted at about 650° F. to 820° F. while employing the same catalyst that is employed in the first stage.

A heavy fuel oil is obtained having a sulfur content of 0.58 weight percent sulfur. The distribution of sulfur in each of the various fractions of the oil undergoing desulfurization is set forth in Table I, below:

TABLE I

| Fraction<br>(percent<br>by wt.) | Feed to first HDS<br>zone                    |                                 | Feed to second HDS<br>zone                   |                                 | Fuel oil product                             |                                 |
|---------------------------------|----------------------------------------------|---------------------------------|----------------------------------------------|---------------------------------|----------------------------------------------|---------------------------------|
|                                 | Sulfur in<br>fraction<br>(percent<br>by wt.) | Fraction<br>(percent<br>by wt.) | Sulfur in<br>fraction<br>(percent<br>by wt.) | Fraction<br>(percent<br>by wt.) | Sulfur in<br>fraction<br>(percent<br>by wt.) | Fraction<br>(percent<br>by wt.) |
| Saturates.....                  | 17.98                                        | 3.42                            | 22.24                                        | 0.80                            | 22.34                                        | 0.49                            |
| Aromatics.....                  | 55.45                                        | 5.04                            | 60.45                                        | 1.12                            | 61.91                                        | 0.56                            |
| Resins.....                     | 16.73                                        | 5.59                            | 13.76                                        | 2.37                            | 12.72                                        | 1.56                            |
| Asphaltenes.....                | 9.84                                         | 6.99                            | 3.55                                         | 4.95                            | 3.03                                         | 3.13                            |

As seen from Table I, it is apparent that in an asphaltic feed containing a total of about 4.09 weight percent sulfur, the sulfur content of such feed is relatively evenly distributed between the saturates, aromatics, resins and asphaltenes. However, after the feed is passed through the first desulfurization zone and the 650° F. E.P. fraction is removed, i.e., at 1.09 weight percent total sulfur, the saturates and aromatics have lost sulfur to the greatest extent, viz, they are down to 0.80 and 1.12 weight percent sulfur respectively, while the resins and asphaltenes have lost sulfur to the least extent, viz, 2.37 and 4.95 percent by weight sulfur, respectively. Finally,

In addition, it is seen from Table I, that the aromatic content of the feed has gone from 55.45 weight percent to 60.45 weight percent after the first stage flashing, and finally up to 61.91 weight percent aromatics in the product. At the same time the weight ratio of aromatics to resins plus asphaltenes increases from about 2 to 1 to about 4 to 1. Thus, Table I clearly illustrates the criticality of providing sufficient aromatics in the asphaltic stream in order to solubilize the resins and asphaltenes and to deagglomerate any asphaltene aggregates so as to permit desulfurization thereof. Likewise, this Table shows the criticality of avoiding an excess of liquid including aromatics, especially saturates, beyond what is required to contribute a solubilizing effect, since such an excess of low-sulfur liquid will only tend to disperse and dilute the sulfur-containing resins, resins and asphaltenes and diminish their chance of contact with the catalyst. It should be further noted that the aromatic content of the feed to the second stage is richer in aromatics, i.e., 60.45 weight percent than is the feed to the first stage, i.e., 55.45 weight percent. This is due, in part to the 650° F. interstage flashing which removes saturates in much greater proportion relative to the aromatics present in the flashed, light oil stream. In each stage, the weight ratio of aromatics to resins plus asphaltenes to accomplish solvation should be at least 1 to 1 and is preferably 1.5 or 2 to 1, and can be 4 or 5 to 1. The aromatics can be present in the feed, can be introduced by recycle or can be produced in situ.

It is further interesting to note that Table I reveals that the saturates, which are flashed off, are the most highly desulfurized fraction and therefore have the least need for passage through the second stage of desulfurization.

The following example illustrates the refractory nature of an asphaltic feedstock when it is attempted to remove more than one percent sulfur without employing the process of the present invention.

#### EXAMPLE 2

A 22 percent reduced Kuwait crude containing an asphalt fraction and 5.43 percent by weight sulfur is

subjected to desulfurization. The initial boiling point of the crude is 556° and the boiling range extends to 1400° F.+. After the sulfur content is reduced to 4.77, the I.B.P. is 514° and the boiling range extends to 1400° F.+.

As desulfurization continues, and the sulfur content is reduced to 1.41, the I.B.P. is 509° with the boiling range extending to 1400° F.+. However, when the sulfur content is reduced to 0.83, the I.B.P. drops 90° F. to 466° F. with the boiling range extending to 1400° F.+.

The results of this run are shown in Table II, below:

TABLE II

| Feedstock                     | Reduction in sulfur content during desulfurization |            |            |            |
|-------------------------------|----------------------------------------------------|------------|------------|------------|
| Sulfur, percent by wt.....    | 5.43                                               | 4.77       | 1.41       | 0.83       |
| Boiling range, ° F.....       | 566-1,400+                                         | 514-1,400+ | 509-1,400+ | 466-1,400+ |
| Desulfurization, percent..... | 12.2                                               | 74.0       | 85.0       | 85.0       |
| ° API.....                    | 6.5                                                | 8.7        | 17.7       | 20.3       |

even after the second stage desulfurization, the only significant sulfur remaining is present in the resins and asphaltenes.

The foregoing data shows that the sulfur content of the feed becomes very refractory at about 74 percent desulfurization. At 12 percent sulfur removal the I.B.P. is

reduced to 415° F., while at 74 percent sulfur removal the I.B.P. is only reduced to 509. However, in order to obtain 85 percent sulfur removal, the I.B.P. is reduced all the way to 466° F. Thus, in single stage operation, hydrocracking begins to predominate over hydrodesulfurization, i.e., carbon-carbon bonds are becoming severed, rather than carbon-sulfur bonds, beyond 74 percent sulfur removal.

The following Table III, below, shows the composition of the feed during the course of the desulfurization reaction:

TABLE III

| Feedstock<br>(percent by<br>wt.) | Composition<br>desulfurization<br>(percent by wt.) | change<br>during<br>desulfurization<br>(percent by wt.) |      |
|----------------------------------|----------------------------------------------------|---------------------------------------------------------|------|
| Desulfurization.....             | 12.2                                               | 74                                                      | 85   |
| Saturates.....                   | 11                                                 | 16.7                                                    | 26.1 |
| Aromatics.....                   | 39                                                 | 41.2                                                    | 56.6 |
| Resins.....                      | 32                                                 | 25.7                                                    | 15.1 |
| Asphaltenes.....                 | 18                                                 | 16.4                                                    | 2.2  |
|                                  |                                                    |                                                         | 1.6  |

The foregoing data show that as the depth of sulfur removal increases, resins and asphaltenes diminish and are converted to saturates and aromatics.

The following Table IV gives a molecular weight comparison of the aromatics, saturates and residuals during the course of desulfurization.

TABLE IV

| Feedstock                     | Molecular<br>weight<br>during desulfurization | change |     |
|-------------------------------|-----------------------------------------------|--------|-----|
| Desulfurization, percent..... | 12.2                                          | 74     | 85  |
| Saturates, M.W.....           | 430.0                                         | 400    | 410 |
| Aromatics, M.W.....           | 490.0                                         | 530    | 400 |
| Total residuals, M.W.....     | 1,080                                         | 590.0  | 490 |
|                               |                                               |        | 420 |

The data in Table IV show that as the depth of desulfurization increases, the molecular weight of the total residuals decrease, but not significantly below the molecular weight of the initially formed saturates and aromatics. This molecular weight pattern further illustrates that during the breaking of carbon-sulfur bonds in the resins and asphaltenes, hydrocarbon fragments are produced which are about in the same molecular weight range as are the feed saturates and aromatics.

## EXAMPLE 3

In order to illustrate the effect of both dilution and concentration of the resins and asphaltenes in the second stage feed upon the second stage desulfurization rate, a 650° F. flash temperature is employed on a feedstock that had been subjected to a single stage of hydrodesulfurization. The asphaltic, flash residue is subjected to a second stage hydrodesulfurization, and it exhibits a desulfurization reaction rate constant of about 85. The desulfurization reaction rate constant is calculated in a conventional manner, i.e.

$$\frac{\text{lb. oil}}{\text{lb. sulfur}} \times \frac{\text{lb. oil}}{\text{hr.-lb. catalyst}}$$

This reaction rate constant can also be expressed as

$$R = \left( \frac{1}{S_p} - \frac{1}{S_f} \right) \text{LHSV}$$

as previously defined.

For comparative purposes, a desulfurized furnace oil having a boiling point in the range of 400° to 650° F. and containing 0.07 weight percent sulfur is added to the residue of the 650° F. flash operation. The furnace oil is comprised of about one-half saturates and one-half aromatics. Upon passing this asphaltic feed through a second stage desulfurization, the desulfurization reaction rate drops to 75. Thus, excessive dilution of the feed to the second stage actually reduces the desulfurization reaction rate, even though aromatics are being added.

For further comparison, 30 percent by weight of a light portion of the second desulfurization stage feed is re-

moved making the feed equivalent to about the residue of an 800° F. flash. In this instance, the reaction rate for desulfurization in the second stage falls to 40 thereby illustrating the effect of inadequate solvation for the resins and asphaltenes. It is clearly evident that the amount of saturates plus aromatics which accompanies the resins and asphaltenes into the second stage has a distinct effect upon the second stage reaction rate, and that too much diluent can have a detrimental effect upon desulfurization reaction rate, just as does too little aromatic solvent.

## EXAMPLE 4

In order to determine the effect of adequate, as contrasted to excessive solubilization of an asphalt-containing feed, a residual, high-boiling feed having an initial boiling point of about 800° F. is charged to a hydrodesulfurization process, and 76.2 percent by weight desulfurization is accomplished. Next, a second sample of the feed is diluted with 30 volume percent of a lower boiling gas oil which had been previously desulfurized to the extent of 90 to 95 percent by weight. The addition of the gas oil, which comprises a high proportion of aromatics, increases the desulfurization to 80.3 percent by weight.

For comparative purposes, a further sample of the feed is diluted with 40 percent by volume of a gas oil and is subjected to desulfurization as before. In this instance, there is a loss in desulfurization activity and the desulfurization drops to 76.3 percent by weight. The development of 64 percent by volume of gas oil reduces the degree of desulfurization even lower to 69.4 percent by weight. The results of these tests are illustrated in Table V below:

TABLE V

| Effect of gas oil dilution           |      |      |      |      |
|--------------------------------------|------|------|------|------|
| Gas oil, percent by vol.....         | 0    | 30.0 | 40.0 | 64.0 |
| Desulfurization, percent by wt.....  | 76.2 | 80.3 | 76.3 | 69.4 |
| Vanadium removal, percent by wt..... | 83.5 | 78.6 | 74.6 | 77.8 |

The foregoing data illustrate the initial advantage that is realized in the hydrodesulfurization of an asphaltic oil due to the solvating power of the aromatics in the gas oil diluent upon the resins and asphaltenes. However, these data further show that this advantage can be more than offset by an excessive amount of diluent, which may disperse the sulfur molecules excessively and thereby reduce the desulfurization reaction rate. Furthermore, an excessive amount of diluent may also reduce the sulfur removal by imparting an excessive increase in space velocity in the desulfurization reactor.

## EXAMPLE 5

A test is performed utilizing in the first and second stages a one-thirty-second inch nickel-cobalt-molybdenum on alumina catalyst. In the first stage the catalyst exhibits a six month life with a start-of-run temperature of 690° F. and an end-of-run temperature of about 790° F. in hydrodesulfurizing a Kuwait reduced crude from 4 to 1 weight percent sulfur at a LHSV of about 0.8. The catalyst life in the second stage is even longer. The one weight percent sulfur effluent from the first stage is flashed to remove 650° F. end point material based on atmospheric pressure and is charged to the second stage with hydrogen to reduce the sulfur level to 0.5 weight percent. The second stage start-of-run temperature is 690° F. and the temperature at 170 days is only 763° F. The test can continue until the temperature is 790° F. Therefore, the first and second stages of this invention can operate for 3, 4, 5, 6 or even 7, 8 or 12 months at a LHSV generally ranging between 0.1 and 10 or preferably between 0.3 and 1.25. The life of the second stage catalyst is longer than the life of the first stage catalyst.

Although the invention has been described in considerable detail with particular reference to certain preferred embodiments thereof, variations and modifications can be effected within the spirit and scope of the invention as

described hereinbefore, and as defined in the appended claims.

We claim:

1. A process for the hydrodesulfurization at a hydrogen partial pressure between 1,000 and 5,000 p.s.i. in a two-zone reaction of a heavy asphaltic feed oil to produce a heavy asphaltic fuel oil product containing propane- and pentane-insoluble asphaltenes and propane-insoluble resins but pentane-soluble resins, comprising passing a sulfur-containing asphaltic hydrocarbon oil feed downflow with hydrogen through a first zone containing at least one bed of hydrodesulfurization catalyst particles  $\frac{1}{20}$  to  $\frac{1}{40}$  inch in diameter at a temperature between 680 and 800° F., the temperature being increased during the reaction to compensate for loss of hydrodesulfurization reaction rate due to catalyst aging, said catalyst particles comprising a Group VI and a Group VIII metal on alumina containing less than one percent silica, withdrawing a first effluent stream from said first hydrodesulfurization zone having a reduced sulfur content, said first effluent stream comprising a light gas fraction including hydrogen sulfide, a light oil fraction containing saturates and aromatics, and a higher-boiling asphaltic fraction containing asphaltenes and resins, separating said light gas fraction and a portion of said light oil fraction from said first effluent stream, said light oil fraction boiling between about 500 and 800° F. when measured at atmospheric pressure, passing said higher-boiling asphaltic fraction containing asphaltenes and resins and the remaining portion of said light oil fraction with additional hydrogen downflow through the second zone containing at least one bed of hydrodesulfurization catalyst particles  $\frac{1}{20}$  to  $\frac{1}{40}$  inch in diameter at a temperature between 680 and 800° F., the temperature being increased during the reaction to compensate for loss of hydrodesulfurization reaction rate due to catalyst aging, said second zone catalyst comprising a Group VI and a Group VIII metal on alumina containing less than one percent silica, operating the catalyst in said first and second zones for at least three months at a liquid hourly space velocity between 0.1 and 10, maintaining the average hydrogen partial pressure in each of said zones sufficiently high that the average hydrodesulfurization reaction rate constant is improved by said two zones of operation and accomplishing a degree of desulfurization with less catalyst as compared with a single zone of operation accomplishing the same degree of desulfurization, withdrawing a second effluent stream from said second hydrodesulfurization zone comprising a low sulfur heavy asphaltic hydrocarbon fuel oil, and recovering said product having less than 1 weight percent sulfur, of said product not less than 50

percent by weight having a boiling point greater than the initial boiling point of the feedstock and not more than 20 weight percent having a boiling point lower than 375° F., said product containing saturates, aromatics, resins and asphaltenes.

- 5 2. The process of claim 1 wherein said average hydrogen partial pressure is between 1400 and 2200 p.s.i.
3. The process of claim 1 wherein said average hydrogen partial pressure is greater in the second zone than in the first zone.
- 10 4. The process of claim 1 wherein said hydrogen partial pressure in the second zone is between about 1400 and 2200 p.s.i.
5. The process of claim 1 wherein the second effluent hydrocarbon contains less than one percent sulfur.
- 15 6. The process of claim 1 wherein said second zone reduces the hydrocarbon stream sulfur content from at least one percent to less than 0.5 percent.
7. The process of claim 1 wherein resins and asphaltenes comprise 5 to 30 percent or more of the feed.
- 20 8. The process of claim 1 wherein at least 75 percent sulfur is removed from the feed in the first zone.
9. The process of claim 1 wherein the second effluent stream contains at least 80 percent by weight of material boiling above the initial boiling point of the feed.
- 25 10. The process of claim 1 wherein not more than 10 percent of the second effluent boils below 650° F.
11. The process of claim 1 wherein the catalyst contains nickel, cobalt and molybdenum.
- 30 12. The process of claim 1 wherein the catalyst age in both zones is at least four months.
13. The process of claim 1 wherein the catalyst age in both zones is at least five months.
14. The process of claim 1 wherein the liquid hourly space velocity is between 0.3 and 1.25.
- 35 15. The process of claim 1 wherein the liquid hydrocarbon effluent from the second zone boiling below 375° F. does not exceed 10 weight percent.

#### References Cited

##### UNITED STATES PATENTS

|              |         |                        |         |
|--------------|---------|------------------------|---------|
| 3,617,525    | 11/1971 | Moritz et al. -----    | 208—211 |
| 3,418,234    | 12/1968 | Chervenak et al. ----- | 208—210 |
| 45 3,530,062 | 9/1970  | Gatsis -----           | 208—89  |
| 3,481,860    | 12/1969 | Borst, Jr. -----       | 208—213 |
| 3,471,398    | 10/1969 | Borst, Jr. -----       | 208—209 |

DELBERT E. GANTZ, Primary Examiner

50 G. J. CRASANAKIS, Assistant Examiner